

## UNITED STATES PATENT OFFICE

2,163,325

## COLOR PHOTOGRAPHY OR CINEMATOGRAPHY

Edgar Sanders-Dolgoruki, London, England, assignor to Truecolour Film Limited, London, England, a British company

No Drawing. Application October 28, 1937, Serial No. 171,593. In Great Britain October 29, 1936

## 5 Claims.

(Cl. 95—2)

The present invention relates to the production of colored records on photographic material of the type comprising a plurality of superposed silver halide emulsion layers differentially sensitized for different regions of the spectrum and each containing color-forming components adapted to react with a diamine or aminophenol developer to produce differently colored images in the different layers.

10 In the manufacture and processing of such material difficulties are encountered owing to the fact that the color-forming components tend to diffuse or bleed from one layer to the other during manufacture or during the development of the material. It has been proposed to overcome this difficulty in such a manner that the color-former or an intermediate product thereof is present in the layer in such a state that as development proceeds it only comes into solution by reaction with the by-products of the developer.

15 For example, a color-former of an acid nature may be insolubilised by conversion into a metal salt, and a color-former of a basic nature may be insolubilised by conversion into a fatty acid salt or a resin acid salt.

20 On the other hand, it has been proposed to employ color-formers of opposite characters in the adjacent layers. Thus, in one layer there may be a color-former of an acid character, while 25 in the adjacent layer or layers a color-former or color-formers of a basic character is/are employed.

25 Another proposal is contained in British patent specification No. 458,400, which consists in employing color-formers containing a chemical group of a substantive character.

30 The processing of such material may be performed by the direct development of the latent images with a diamine or similar color-forming developer, or by the production of reversed images by first developing the material with a developer such as metol which is incapable of reacting with the color-formers, removing the developed images and redeveloping the remaining 35 silver halide with a color-forming developer to produce reversed color images in the different layers.

35 In the production of reversed images the material can be left in the solution of the color-forming developer as long as is required for the reason that no damage can occur to the image in a layer which is already fully developed, while development in the other layer or layers continues.

40 In the processing of such a photographic material to form a record of a negative character by color-developing the latent images produced on exposure, the difficulty is encountered that development tends to proceed at a different rate in the different layers, so that it is difficult to obtain 45 the desired gradation values for the different

colored images. If the color development were permitted to proceed to "gamma infinity," a considerable amount of color "fog" would be formed in those layers in which the color-development proceeds rapidly.

5 It has now been found that the difficulties met with in the direct processing of the latent images in such emulsion layers containing color-formers may be overcome by a method which in accordance with the invention, consists in first 10 developing the said latent images with a developer which is incapable of affecting the color-formers in such layers, removing the unaffected silver halide, converting the developed silver images into redevelopable silver salt images and 15 redeveloping the material in a developer which is capable of reacting with the color-formers in the layers.

20 It has heretofore been proposed in British patent specification No. 447,092 to process a photographic material, embodying several emulsion layers which do not contain color-formers, by first developing the layers to form silver images therein, fixing and washing the material and then bleaching the silver images to redevelopable 25 silver salt images, after which the layers are redeveloped with a developer containing a color-forming component in order that all the latent images in said layers can be color-developed to one color. Subsequently the material was inserted in a loaded bleaching bath to bleach some 30 of said images and redeveloped in another color-forming developer to produce a different color in those layers that were bleached, and this procedure was repeated with different color-forming 35 developers until the images in all the layers had been processed to different colors.

40 The present invention is restricted to the processing of photographic material in which at least some of the layers contain color-forming components prior to exposure, which components are capable of reacting with the oxidation products of suitable developers to form differently colored images in such layers at a single operation.

45 In carrying the invention into effect a photographic material may be employed comprising three photographic emulsion layers which may either be disposed all on one side of a support 50 or two may be disposed on one side and a third on the other side of the support, and such layers may contain suitable color-formers of such a character in accordance with the prior art that diffusion or bleeding from one layer to the other is minimised. The said layers or some of them 55 are differently sensitised for different regions of the spectrum, and if desired between some or all of said layers known decolorisable filter layers may be provided, and in addition, if desired, at the rear of the material may be provided an anti- 60

halation backing which is capable of removal or decolorisation by the treatment baths.

After the exposure of such material, the first step in processing is to develop the latent images in all the layers to silver in a developer which is incapable of reacting with the color-formers in the emulsion layers; such developer is for example the following metol developer:—

|                   |     |       |
|-------------------|-----|-------|
| Metol             | gm. | 3     |
| Sodium sulphite   | do  | 30    |
| Sodium carbonate  | do  | 45    |
| Potassium bromide | do  | 0.5   |
| Water, q. s.      | cc. | 2,000 |

15 The unaffected silver halide in the layers is then removed in a solution of sodium thiosulphate and the material thoroughly washed. The silver images in the layers are then converted into a silver salt which is capable of redevelopment with a color-forming developer, in some cases after re-exposure to light. A suitable silver salt for this purpose is silver ferrocyanide in which case the following bleach bath could be employed:—

|                        |     |     |
|------------------------|-----|-----|
| Potassium ferricyanide | gm. | 20  |
| Ammonia 28% solution   | cc. | 20  |
| Water, q. s.           | do  | 100 |

15 The material may be re-exposed to light, although this step is not normally necessary, and inserted in a developer, the oxidation products of which are adapted to react with the color-formers in the layers at the points where development of the silver salt occurs, to produce colored images in the different layers; such color-forming 20 developers are well known in the art but the following diethylparaphenylenediamine is quoted by way of example only:—

|                                           |     |       |
|-------------------------------------------|-----|-------|
| Diethylparaphenylenediamine hydrochloride | gm. | 0.82  |
| Sodium sulphite (crystals)                | do  | 5     |
| Potassium carbonate (anhydrous)           | do  | 20    |
| Water, q. s.                              | cc. | 1,000 |

45 Of course, the photographic material may comprise more than three photographic emulsion layers and all or only some of said layers may contain color-formers. Thus, a material suitable for a four-color process in which a fourth emulsion layer is provided intended to give a black and white image, may comprise three layers containing suitable color-formers while the fourth layer may be an ordinary photographic emulsion. Moreover, whether the material comprises 50 three or four emulsion layers some of the layers in which colored images are produced may be processed by other methods than those described herein.

55 Thus again, a photographic material comprising two emulsion layers on one side of the support and a single layer on the other side of the support may contain different color-formers in the said two layers, while the layer on the other side of the support may be an ordinary photographic emulsion, a color image being formed therein during the processing by other known processes of color development wherein the color-former is mixed with the developer, by dye-toning, chemical toning or otherwise.

I claim:

70 1. A method of processing a photographic material comprising a plurality of superposed silver

halide emulsion layers containing color-forming components to produce differently colored images in the different layers comprising developing the latent image in all of said layers with a developer incapable of affecting the said color-formers, removing the unaffected silver halide from said layers, converting the developed silver images into silver salt images which are capable of redevelopment and developing said silver salt images with a developer, the oxidation products 10 of which are capable of reacting with the said color-formers to produce differently colored images in the layers.

2. A method of producing a non-reversed color record on a photographic material comprising 15 superposed silver halide emulsion layers sensitive to different spectral regions and containing color-forming components to partake in the production of the colored images in said layers which consists in developing the latent images in said 20 emulsion layers to silver with a developer which does not affect the color-formers, removing the unaffected silver halide from said layers, converting the developed silver images into developable silver salt images and then developing said 25 silver salt images to different colors by a single treatment with a developer the oxidation products of which are capable of reacting with the said color-formers to produce colored images in the different layers.

3. A method of producing a multi-color photographic record by a process which does not include reversal on a photographic material comprising several superposed emulsion layers containing color-forming components adapted to react with a paraphenylenediamine developer which consists in developing silver images in all of said layers with a developer which does not affect the color-forming components, removing the unaffected silver halide from said layers, converting the developed silver images into redevelopable silver salt images and redeveloping the material in a paraphenylenediamine developer to produce differently colored images in all of said layers.

4. A method of producing a non-reversed multi-color photographic record on photographic material comprising a plurality of superposed silver halide emulsion layers containing color-forming components which consists in developing 50 silver images in all of said layers, removing unaffected silver halide in said layers, converting said silver images into developable silver salt images, developing the latter images in a developer capable of reacting with said color-forming 55 components to produce differently colored images in said layers and finally removing developed silver from said layers.

5. A method of producing a non-reversed multi-color photographic record on photographic 60 material comprising a plurality of superposed silver halide emulsion layers containing color-forming components which consists in developing silver images in all of said layers, removing the unaffected silver halide from said layers, converting the developed silver images into silver ferro-cyanide and developing the latter images with a developer capable of reacting with the color-forming components to produce differently colored images in said layers.

EDGAR SANDERS-DOLGORUKI.